

# UNITED STATES PATENT OFFICE.

AUGUSTE J. ROSSI, OF NIAGARA FALLS, NEW YORK, ASSIGNOR TO THE TITANIUM ALLOY MANUFACTURING COMPANY, OF NEW YORK, N. Y., A CORPORATION OF MAINE.

## PROCESS FOR BLEACHING ARTICLES.

1,080,718.

Specification of Letters Patent.

Patented Dec. 9, 1913.

No Drawing.

Application filed January 31, 1912. Serial No. 674,544.

To all whom it may concern:

Be it known that I, AUGUSTE J. ROSSI, a citizen of the United States, and a resident of Niagara Falls, in the county of Niagara and State of New York, have invented certain new and useful Improvements in Processes for Bleaching Articles, of which the following is a specification.

My present invention relates to what is broadly termed "bleaching," including the "discharging" from fabrics of undesired natural or artificial coloring matters or pigments, or the "restoring" of the latter when undesirably dimmed by undue oxidation.

The objects of my invention comprise the economical, effective, and less destructive bleaching of materials, also the economical and simple production of a bleaching solution competent for the purpose.

I am aware that sulfur dioxid and chlorin, or what is commonly known as "bleaching powder," have heretofore been employed in bleaching fabrics. But while free chlorin may be said to bleach certain fabrics quite completely, its destructive action on, or undesirable alteration of, fibers of animal origin, silk for instance, renders its use thereon hazardous and in most cases undesirable or impossible.

The use of sulfur dioxid for bleaching is also, in many instances, far from satisfactory, some fabrics treated therewith, particularly those previously dyed, coming out less purely white than is desirable, and showing off, when ironed, too many traces of their original colors.

By the cautious and skilful use of certain well known bleaching powders, such for instance as depend largely on chlorin liberated from hypochlorites, better results are often obtained, but the presence of such chlorin causes such deterioration in the fiber and appearance of the silken portions of the fabric as to cause loss to the manufacturer.

I have long shared with others the conception that chlorid of titanium might possibly be used with advantage as a substitute for the aforesaid bleaching agents, and have experimented in hopes of realizing this. To this end I produced the tetrachlorid of titanium,  $TiCl_4$ , by the well known method which consists in passing chlorin gas over a mixture of carbon and titanic acid heated to redness, thereby obtaining a yellowish liquid

smelling strongly of chlorin because containing free chlorin in solution. On applying this solution experimentally to some textiles, I found them bleached to an extent, but realized that, owing to its free chlorin, it could not be used to bleach materials of animal origin such as silk and wool, on account of the aforesaid deteriorating action of such chlorin on such materials, i. e. its impairing their strength and brilliancy, etc. Realizing that these characteristics and results prohibited the use of such a solution on materials other than of vegetable origin, such as cotton, etc. I resorted next to well known methods by which I was enabled to eliminate free chlorin therefrom to an extent. On applying the solution thus freed I found that it had no bleaching effect, from which I infer that the tetrachlorid of titanium is not by itself a bleaching agent.

I have now discovered that a titanous chlorid such as titanium sesquichlorid,  $Ti_2Cl_3$ , is, if in my solution hereinafter described, a bleaching agent uninjurious to animal substances such as silks, or wool, etc., whether in raw condition, or manufactured as textiles, etc.

My said solution containing the desired sesquichlorid of titanium in any required amount may be economically and readily produced by dissolving, in hydrochloric acid at normal temperature, an alloy of iron and titanium commonly known as ferro-titanium. The said solution so produced is exceptionally well adapted to bleaching purposes, not only because of its said content of said sesquichlorid, but also because of absence therefrom of free chlorin injurious to animal substances, this being due to its content of ferrous chlorid which is not only itself non-injurious but also contributes to the stability of the solution.

I produce said solution as follows:—In a vessel lined preferably with porcelain or like resistant material, I dissolve, at below boiling temperature, in hydrochloric acid diluted with its weight of water or less, an alloy of iron and titanium as high in titanium as desired, for example the alloy for which were granted to me Letters Patent No. 648,439, dated May 1, 1900. The resulting liquor should be of a violet color, thus indicating that the sesquichlorid of ti-

tanium has been formed. I next filter the liquor to remove therefrom such small quantities of silica, carbon, or other impurities, including the titanium oxid which should be formed but to a small extent. Ordinary filter presses, or any other similar contrivances, can be used with advantage for this purpose. The liquid thus filtered is then ready for use.

10 As will be readily understood by those skilled in the art, the respective proportions of the respective ingredients of the charge in producing said solution will depend upon the respective ascertained characteristics 15 and proportions of each; that is to say the amount by weight of commercial hydrochloric acid charged will, in each case, depend upon its HCl content and upon the amount of the latter required to satisfy the 20 respective chemical affinities therefor of all the iron and titanium in the charge.

Careful tests have demonstrated that the presence of the chlorid of iron interferes in no respect with the bleaching properties of 25 my said solution, these being exceptionally perfect, and non-injurious to the materials of animal origin to which applied; also that it is characterized as containing substantially no free chlorin; also that it is very 30 notably stable as compared with previous solutions containing compounds of chlorin. Its chlorids appear to part with their chlorin only in proportion as the bleaching proceeds, and when sufficiently proximate to the

35 coloring matter with which it promptly combines, thus precluding the presence of free chlorin in the solution at any stage. This comparative stability of my solution seems attributable only to its content of 40 ferrous chlorid which principally distinguishes it from all previous solutions containing titanous chlorids, for example such as have heretofore been suggested as able to discharge color from fabrics. It seems 45 that the titanous chlorids of such previous solutions have, owing to their nature and environment, proved too, if not prohibitarily, unstable, their titanium content tending to separate and combine with oxygen present to 50 form titanic acid, thus prohibitarily liberating in the solution free chlorin to injure animal substances if thereby treated; whereas, in my said novel solution, such free chlorin if any so liberated combines promptly 55 with the ferrous chlorid present to form ferric chlorid, whereby free chlorin is substantially prevented from reaching and deteriorating the bleaching animal fibers, such as that of silk, which would otherwise be 60 ruined thereby.

The methods of applying my said solution to the materials treated thereby will of course be readily understood by those skilled in the bleaching art. The violet solution

is of course diluted with water to meet the 65 special requirements of the particular materials or particular dyes therein contained, such dilution causing the violet color to assume lighter shades in proportion to the water added. Should the solution in any 70 case prove too strongly acid, its acidity may be counteracted by additions of any proper alkali, such as ammonia for example. To avoid injury to the materials it is of course preferable that the solution employed 75 should be but slightly acid. The solution will be applied to the materials treated in substantially the same way as any other solution employed for bleaching purposes. Such methods of application are too well 80 understood to require description here. For instance the usual bleaching vats are employed, the solution charged thereinto and the materials soaked therein as usual, or the solution may be otherwise applied in 85 any convenient manner. The temperatures employed will depend upon the preference and experience of the individual operators. Normal temperatures involve longer exposure to the solution and higher temperatures shorter exposure as will be well understood. It is preferable to avoid boiling temperature except in cases in which the solution is very considerably diluted. It goes without saying that the fabrics, after 90 application thereto of the solution, are thoroughly washed, etc., according to the usual procedure of the art.

Applications of my said bleaching solution, derived as aforesaid from an iron titanium alloy containing about 16 per cent. titanium, made to a cotton fabric of slightly lavender color containing stripes of silk of a deeper shade gave the following results. Said fabric, boiled in my said solution diluted ten times with water to meet the special requirements of this particular fabric was rapidly bleached a pure white, notwithstanding which the brilliancy of the silk stripes was unimpaired. Other specimens of 100 the same fabric, treated as usual with sulfur dioxide solutions emerged not completely bleached, the white having a grayish blue hue prohibiting the use thereof as a 105 white fabric and objectionable for dyeing in certain delicate light colors. Other specimens of the same fabrics treated as usual with chlorin, or bleaching powders, above referred to, presented a deteriorated appearance, and, though nearer to pure white, their 110 silk stripes had lost much of their original brilliancy.

It is preferable in my experience that the ferro-titanium employed should contain not less than 16 per cent. of titanium, and be dissolved as aforesaid in hydrochloric acid diluted by about its own weight of water to 115 produce, prior to further dilution for use,

an initial solution containing not less than about 25 per cent. of the sesquichlorid of titanium.

Maintenance of the bath at substantially normal, *i. e.* below boiling, temperature is, I have discovered, essential in order to produce the desired sesquichlorid of titanium from the ferro-titanium treated under the conditions mentioned. My experiments have demonstrated that if the temperature of the bath rises to approximately, or above, boiling, the titanium content goes to make titanium oxid, more or less precipitated, which, like other compounds of titanium except the sesquichlorid, appears unable to bleach, as desired, the fabric or other material treated, thus wasting the chlorin content notwithstanding surplus free chlorin so liberated is promptly taken up by the ferrous chlorid present as aforesaid.

It will of course be understood that my said method, and my solution containing both titanous and ferrous chlorids, are equivalently applicable, as above described, to not only "bleaching" specifically, but also to the "discharging" of colors previously artificially applied, and also to the "restoring" of colors. In each of these applications the reducing action of the titanous chlorid is similarly relied upon; *i. e.* in bleaching it deoxidizes as required to improve the appearance of the fabric wherever it has been undesirably affected by oxidizing agents; in discharging, it also deoxidizes to remove the color from previously applied artificial dyes; in restoring, it also deoxidizes to restore original color to portions of the fabric which, by reason of previous finishing or bleaching treatments, have been unduly oxidized and consequently dimmed or altered.

What I claim as new and desire to secure by Letters Patent is the following, viz:—

1. The method of bleaching materials which comprises applying thereto a solution containing sesquichlorid of titanium ( $Ti_2Cl_6$ ) and ferrous chlorid. 45

2. The method of bleaching materials which comprises applying thereto a solution containing titanous chlorid and ferrous chlorid. 50

3. The method of bleaching materials which comprises dissolving titanium and iron in dilute hydrochloric acid, filtering the resulting solution, and applying it to said material. 55

4. The method of bleaching materials which comprises dissolving an alloy of iron and titanium in dilute hydrochloric acid, filtering the resulting solution, and applying it to the said material. 60

5. The method of bleaching materials which comprises dissolving in dilute hydrochloric acid at below normal boiling temperature an alloy of iron and titanium, filtering the resulting liquor to remove therefrom impurities including titanium oxid, and carbon, and then applying it to said materials. 65

6. The method of bleaching materials which comprises dissolving titanium and iron in dilute hydrochloric acid at below normal boiling temperature, filtering the resulting liquor to remove therefrom impurities including titanium oxid, and carbon, and then applying it to said materials. 70

AUGUSTE J. ROSSI.

Witnesses:

WALTER D. EDWARDS,  
PHILIP C. PECK.